

J. P. CRANE.

COMPOSITION CONTAINING ANNEALED STEEL WOOL AND RUEBER.

APPLICATION FILED MAR. 18, 1911.

1,112,772.

Patented Oct. 6, 1914.

FIG. 1.



FIG. 2.



Witnesses:

Leopold D. Marin.  
F. E. Brown.

James P. Crane, Inventor  
by Jno. G. Elliott, Secy.

# UNITED STATES PATENT OFFICE.

JAMES P. CRANE, OF CHICAGO, ILLINOIS.

## COMPOSITION CONTAINING ANNEALED STEEL-WOOL AND RUBBER.

1,112,772.

Specification of Letters Patent.

Patented Oct. 6, 1914.

Application filed March 18, 1911. Serial No. 615,254.

*To all whom it may concern:*

Be it known that I, JAMES P. CRANE, a citizen of the United States, and a resident of Chicago, in the county of Cook and State of Illinois, have invented certain new and useful Improvements in Compositions Containing Annealed Steel-Wool and Rubber, of which the following is a full, clear, and exact specification.

This invention relates to improvements in compositions consisting of vulcanized rubber and steel wool in which the characteristics, form and material, peculiar to steel wool fibers, are utilized to bind and reduce the lateral expansion of its wearing surface without impairing the resiliency of the rubber and the frictional resistance of these fibers as a means rendering such surfaces non-slipping and non-skidding, whereby a composition is produced which is especially adapted for use in the construction of automobile and bicycle tires, hoof pads, shoe heels and other articles, wherein a substantial resiliency, reduction in the frictional wear of the rubber and the non-slipping and non-skidding of their treads are essential for obtaining the best possible results.

Steel wool is a well recognized article of commerce, every fiber of which is thread-like and has an irregular and triangular shape, giving steel wool a peculiar quality for rubbing and other purposes, and requiring for its production specially manufactured and prepared wire and expensive special machinery, tools and skilled labor, and is so different in the material of which it is composed, manner of its production, form and appearance to the eye and touch, and in its characteristics and uses for which it is adapted from lead wool or other fibers or turnings, that it is clearly distinguishable from and is not to be confused with same.

The animal wool-like curled form or kinkiness of the fibers of steel wool is produced by a process of tempering them concurrently with their cutting, and to such a hardness and brittleness that they break when subjected to the pressure necessary when vulcanizing layers of steel wool alternately with sheets of rubber in a mold, and also by the pressure of the rollers of an ordinary mixing machine, commonly used for mixing the fibers with raw rubber compound in a dough-like state, and finally reducing the composition to a slab or sheet-like form before vulcanizing it, as must be for the

purposes of its uses. In other words, the pressure necessary for the thorough incorporation and desired distribution of the steel wool fibers throughout the rubber is such that they are not only broken in two, but into lengths so short that instead of wearing off with the rubber they are discharged therefrom by the resistance of the opposing friction to which they are subjected. Furthermore, owing to the resiliency of these steel fibers, very many of them unavoidably present a side wearing surface forming loops over the surface of the rubber, as it continues to wear away, which not only reduce the effectiveness of the steel fibers for preventing slipping and skidding, but that the fibers are wasted through the breaking of these loops, and not only by their breaking off at the surface of the rubber, but quite frequently inwardly of the surface, and to this extent exposing the rubber to unprotected wear.

The object of this invention is to reduce the fibers of steel wool to a condition substantially reducing their tendency to break, and, thereby maintaining them of the desired length, in a composition composed of rubber and steel wool, and yet retain steel wool fibers in the condition necessary for their effective operation as a binder preventing an undue lateral expansion under pressure of a rubber and steel wool composition when used for the purposes before referred to.

Another and important object of my invention is to reduce the fibers of steel wool to a condition by which it is both practicable and possible to have the fibers disposed in a general longitudinal direction in the rubber, and thereby compel their end presentation to an opposing frictional surface, best resisting the wearing away of the rubber, and insure the effectiveness of steel wool fibers for preventing the slipping and skidding of a rubber surface, and retarding its wearing away when opposed to frictional surfaces, without reducing the effectiveness of steel wool fibers as a binder for resilient rubber, and an undue expansion thereof of force directed against it.

With these ends in view, my invention finds embodiment in certain features of novelty in the construction, combination, and arrangement of parts by which the said objects and certain other objects are herein-after attained, all as fully described with

reference to the accompanying drawings, and more particularly pointed out in the claims.

In said drawings:—Figure 1 illustrates, 5 in perspective view, a slab of a rubber and steel wool compound showing the appearance of a tempered steel wool therein; and, Fig. 2 is a similar view of another slab of a compound of steel wool and rubber showing 10 the appearance and arrangement of the steel wool fibers following the use of the invention of my present process.

In carrying out my invention, I subject 15 a mass of steel wool to any ordinary annealing process, drawing the temper of the fibers until they are reduced to such a state of flexibility that when mixed with a mass of 20 raw rubber composition, of dough-like consistency, and the mass is then repeatedly passed in the same direction between the 25 rollers of a mixing machine commonly and generally employed for mixing rubber with its fluxes and alloys, the fibers will not become unduly broken, and will dispose themselves generally in a longitudinal direction 30 of the resulting slab or sheet, and generally retain this arrangement throughout the vulcanizing process and subsequent use.

The degree to which the fibers are annealed may be such that when the mass of 35 fibers is pulled by hand or combed to a sheet-like form, they will be disposed in a general longitudinal direction, and retain this general direction when placed between sheets of raw or partly cured rubber, and throughout 40 the vulcanization of the mass under pressure in molds for that purpose.

In practice the fibers are annealed to a degree providing for their general longitudinal disposition in the rubber and yet re-

tain their lengths sufficient to provide binding the rubber against lateral expansion, and that the frictional wear upon the fibers may be generally against their ends, and not substantially against their side faces 45 until the rubber is so worn down that the compound has no further value for the purposes and uses to which it is applied.

Practice has demonstrated that when the fibers of steel wool are annealed, as above described, they may be brought to assume and remain disposed in the rubber in a general longitudinal direction, successfully reducing the tendency to be punctured by nails and 50 glass, when in the form of automobile and 55 bicycle tires, or an injurious cutting of shoe heels, soles, hoof pads, etc.

Having described my invention, what I claim and desire to secure by Letters Patent, is:—

1. A new compound of rubber and steel wool consisting of vulcanized rubber and annealed fibers of steel wool incorporated therewith throughout the mass.
2. A new compound of rubber and steel wool consisting of resilient vulcanized rubber and annealed steel wool fibers incorporated therewith throughout the mass.
3. A new compound of rubber and steel wool consisting of resilient vulcanized rubber and annealed fibers of steel wool incorporated with and disposed in a general longitudinal direction throughout the mass.

In witness whereof, I have hereunto set my hand and affixed my seal, this 3rd day 75 of March, A. D. 1911.

JAMES P. CRANE. [L. S.]

Witnesses:

F. E. BROM,  
JNO. G. ELLIOTT.